

# UNITED STATES PATENT OFFICE.

BENJAMIN B. LEACH, OF HIGGINSVILLE, MISSOURI.

## LIQUID COATING COMPOSITION.

1,413,599.

Specification of Letters Patent. Patented Apr. 25, 1922.

No Drawing.

Application filed November 29, 1921. Serial No. 518,655.

*To all whom it may concern:*

Be it known that I, BENJAMIN B. LEACH, a citizen of the United States of America, and resident of Higginsville, in the county 5 of Lafayette and State of Missouri, have invented certain new and useful Improvements in Liquid Coating Compositions, of which the following is a specification.

This invention relates to a liquid coating 10 for treating surfaces that have been painted in order to cause the paint to dry, and it may also be employed as a filler or coating for iron pipe that has been smeared with tar to such an extent as to render the tar hard and 15 capable of receiving a coat of paint or the like.

The liquid is also of great utility in treating sticky wood or leather to condition it for receiving a coat of paint.

20 A still further object of this invention is to produce a drier of the character indicated which comprises comparatively few inexpensive ingredients, the product from which will prove satisfactory in use as a drier of 25 paint, tar or the like.

In carrying the invention into practice, glue, alum and water are employed, the same being commingled and agitated until the glue and the alum have been dissolved, after which the liquid is ready for use as a coating. 30

In producing the compound, I prefer to employ the ingredients in the following proportions, viz:

Glue 4 parts; alum 1 part, and boiling water 16 parts. 35

The coating is employed as a drier by applying thin coatings of it to the article to be treated, and since the action is almost instantaneous, the glue hardens and the paint over which it is applied becomes protected, and when applied to posts or pipes 40 having tar pitch on them, the said tar pitch is hardened to a degree that will receive and hold paint.

I claim:

45 The herein described drier composition consisting of 1 part of alum; 4 parts of glue and 16 parts of boiling water.

BENJAMIN B. LEACH.